

# United States Patent

Liehe et al.

[15] 3,657,127

[45] Apr. 18, 1972

[54] UREIDO THICKENED GREASE

[72] Inventors: Hubert J. Liehe, Whiting; Wilbur L. Hayne, Hammond, both of Ind.

[73] Assignee: Standard Oil Company, Chicago, Ill.

[22] Filed: July 25, 1969

[21] Appl. No.: 845,028

[52] U.S. Cl.....252/49.6, 252/51.5 R, 252/51.5 A

[51] Int. Cl. ....C10m 5/20

[58] Field of Search .....252/25, 51.5 R, 51.5 A, 49.6

2,710,840 6/1955 Swakon et al.....252/51.5

Primary Examiner—Daniel E. Wyman

Assistant Examiner—I. Vaughn

Attorney—Arthur G. Gilkes, William T. McClain and David B. Koss

[57] ABSTRACT

Certain properties of lubricant greases prepared by thickening a lubricating oil with a thickener prepared by reacting stoichiometric amounts of an abietyl amine and a polyisocyanate are improved by incorporating in such lubricant greases an excess of the polyisocyanate.

5 Claims, No Drawings

[56] References Cited

UNITED STATES PATENTS

3,015,625 1/1962 Rosskopf et al.....252/51.5

1  
UREIDO THICKENED GREASE

BACKGROUND OF THE INVENTION

U.S. Pat. No. 3,015,625 issued Jan. 2, 1962, to R. J. Ross-  
cup and H. J. Liehe, the disclosure of which is incorporated  
herein by reference, describes and claims lubricant greases  
prepared by thickening a lubricating oil with a thickener  
prepared by heating a mixture of an abietyl amine and a  
polyisocyanate in the equivalent weight ratio of 1:1. Usually  
the ureido thickened grease contains a slight stoichiometric ex-  
cess of the amine. Greases prepared with such ureido com-  
pound thickeners exhibit excellent lubricating properties at  
elevated temperatures. However, because the cost of prepar-  
ing such greases may be higher than the cost of preparing  
greases with other thickeners, it is desirable to find a method  
of decreasing such cost. One way of accomplishing this would  
be by improving the yield of a grease product by decreasing  
the penetration of the grease product for a given thickener  
content.

SUMMARY

In accordance with the present invention, the yield and  
other properties of lubricant greases prepared with an ureido  
compound thickener of the general Formula (I) of U.S. Pat.  
No. 3,015,625, *supra*, are improved by incorporating in the  
finished grease base an excess, in amounts of from about 0.05  
percent to about 2 percent, of the stoichiometric amount of the  
polyisocyanate required for the formation of the ureido com-  
pound thickener. Preparation of the ureido compound  
thickener in the presence of excess polyisocyanate will  
prevent the formation of grease of the proper consistency.

Accordingly, lubricant grease compositions of the present  
invention comprise a lubricating oil thickened to the desired  
consistency, i.e., penetration, with from about 2 percent to  
about 25 percent of at least one ureido compound of the  
general Formula I, and from about 0.25 percent to about 0.5  
percent stoichiometric excess of a polyisocyanate as  
hereinafter defined.

The ureido compound thickeners used in preparing the  
grease base of the present invention have the general formula



where R and R'' are the same or different abietyl radicals  
selected from the group consisting of a dehydroabietyl radical,  
a dihydroabietyl radical, and tetrahydroabietyl radical and  
mixtures thereof and R' is an alkylene radical or substituted  
alkylene radical of from one to about 30 carbon atoms or an  
arylene radical or a substituted arylene radical. The radicals  
R, R' and R'' can contain substituents such as, for example, al-  
kyl, alkoxy, cyano, aryl, hydroxy, carboxy, halogen, nitro and  
other substituent groups. The alkylene radical can be straight  
and/or branched chain, and the arylene radicals can be  
mononuclear or polynuclear such as phenylene, biphenylene,  
naphthylene, anthrylene and phenanthrylene radicals. The  
terms "alkylene and arylene radicals" as used herein and in  
the appended claims include substituted alkylene radicals and  
substituted arylene radicals.

The general structural formula of the above-named abietyl  
radicals are:



2



The ureido compound can be prepared by heating a mixture  
of an abietyl amine such as hereinafter named and a polyiso-  
cyanate in the equivalent weight ratio of 1:1, at a temperature  
within the range of room temperature (about 70° F.) to about  
450° F.

The ureido compound thickened grease can be prepared by  
preforming the ureido compound as described in Example I of  
U.S. Pat. No. 3,015,625, *supra*, incorporating the ureido com-  
pound in the oil vehicle, and adding the excess polyisocyanate.

Another method of preparing the grease is to form the  
ureido compound *in situ* in the oil vehicle. In the *in situ*  
method, the desired amount of the polyisocyanate is placed in  
a high temperature grease kettle, or other suitable heating  
equipment, containing a major proportion of the liquid lubri-  
cant vehicle to be used and the mixture heated to effect solu-  
tion. To the heated solution is added the hydroabietylamine  
and the balance of the oil or a solution of the hydroabietylamine  
in the balance of the liquid lubricant vehicle and the mixture  
heated to a temperature of about 200° F. to 450° F. and main-  
tained at said temperature until the product increases to the  
desired consistency. The temperature at which the mixture  
sets-up depends largely upon the nature of the liquid lubri-  
cant vehicle employed. When using a  
hydrocarbon oil such as a petroleum oil the mixture sets-up or  
reaches the desired consistency when the temperature reaches  
350°-400° F., while when using a synthetic oil, such as a dial-  
kyl ester of a dibasic carboxylic acid, such as di-isooctyl aze-  
late, dialkyl sebacate, etc., the desired consistency is obtained  
by heating to 220°-320° F. After the formation of the ureido  
compound, the excess amount of the polyisocyanate is then  
added to the grease mix and the product finished by cooling  
and milling.

Still another method of making the grease is to first prepare  
a concentrate of the ureido compound in an oleaginous vehi-  
cle, mixing the preformed ureido compound concentrate with  
the necessary amount of the lubricant vehicle to give a grease  
product containing the desired amount of the ureido  
thickener, and then adding the desired amount of excess  
polyisocyanate. If desired, the excess polyisocyanate may be  
incorporated in the preformed ureido compound concentrate.

The ureido compound concentrate can be suitably prepared  
by maintaining a solution of the abietyl amine and an oil, for  
example a petroleum oil of suitable viscosity, at about 80° F.,  
and a solution of the polyisocyanate and the oil at about 200°  
F., and combining the two solutions in a spray nozzle and per-  
mitting the sprayed droplets of reacting solutions to fall freely  
in a spray tower. By controlling the rate of flow with respect to  
the internal volume of the spray nozzle, the reacting solution is  
discharged before crystallization occurs, and most of the  
precipitation of the resultant reaction product occurs during  
the fall through the spray tower. The precipitated droplets are  
suitably collected in shallow pans at the bottom of the spray  
tower and the collected material permitted to cool to ambient  
room temperature in a quiescent state. Concentrates from

about 25 percent to about 60 percent of the ureido compound in oil can be prepared by the above method, although obviously the method is equally suitable for the preparation of smaller or larger amounts of the ureido compound in oils. The so-called spray technic above described, is described and claimed in U.S. Pat. No. 2,925,387, to T. Traise et al., which is incorporated herein by reference.

Lubricating greases can be readily prepared with the above described ureido concentrates by charging the ureido concentrate to a mixing kettle, adding a portion of the oil vehicle thereto, while stirring and raising the temperature to about 200° to 250° F., preferably about 200° F. At this temperature, the remaining portion of the oil vehicle required to bring the grease to the final desired thickener concentration is added, and the temperature of the mix raised to about 350° to 410° F., preferably about 385° F., at which temperature it is held for about 5 to 60 minutes, preferably about 30 minutes. The grease is then cooled to about 175° to 300° F., preferably about 200° F., the excess amount of the polyisocyanate added, and such additives as desired then incorporated in the product. The grease is then passed through a colloid mill and packaged.

Examples of abietyl amines, i.e., aliphatic amines attached to an alicyclic structure, which can be used in the preparation of the above described ureido compounds are dehydroabietyl amine, dihydroabietyl amine and tetrahydroabietyl amine or mixtures of such amines. A particularly well suited amine is a product marketed by Hercules Powder Company as "Amine 750." This product is prepared by the catalytic hydrogenation of "Rosin Nitrile D" prepared by the action at elevated temperatures of ammonia on hydrogenated rosin. Distilled and undistilled grades are available as "Amine 750" and "Amine 751." The "Amine 750" is a mixture of abietyl amines as follows:

Dehydroabietyl amine

Dihydroabietyl amine

Tetrahydroabietyl amine

The polyisocyanate used may be an aliphatic or an aromatic polyisocyanate. Examples of suitable polyisocyanates are tolylene diisocyanate; p,p'-diisocyanate biphenyl; 1,4-diisocyanato-benzene; p,p-diisocyanato-diphenylmethane; 1,6-diisocyanato-hexane; 1,12-diisocyanotododecane; 1,3,5-benzene-triisocyanate; naphthylene diisocyanate; bitolylene diisocyanate; tris-p-isocyanato-phenylmethane; etc.

Oleaginous lubricant vehicles which can be thickened with the herein described polyureido compounds to form greases of the present invention can be silicone polymer oils, mineral lubricating oils, synthetic hydrocarbon lubricating oils, synthetic lubricating oils such as polyalkylene glycols and their derivatives, high molecular weight esters of dicarboxylic acids, polyfluoro derivatives of organic compounds such as the trifluorovinyl chloride polymers known as "Fluorolube" (made by Hooker Chemical Company) and the trifluorochloroethylene polymers, known as example, Kel-F-0" (made by The M. W. Kellogg Company), and other lubricant vehicles.

Other oleaginous vehicles which may be employed are, for example, mineral oils in the lubricating oil viscosity range, i.e., from about 50 S.S.U. at 100° F. to about 300 S.S.U. at 210° F. These mineral oils may be suitably solvent extracted, with phenol, furfural, B,B'-dichlorodiethyl-ether (Chlorex), liquid SO<sub>2</sub>, nitrobenzene, etc. Synthetic lubricating oils resulting from polymerization of unsaturated hydrocarbons or other oleaginous materials within the lubricating oil viscosity range such as high molecular weight polyoxyalkylene compounds such as polyalkylene glycols and esters thereof, aliphatic diesters of dicarboxylic acids such as the butyl, hexyl, 2-ethylhexyl, decyl, lauryl, etc., esters of sebacic acid, adipic acid, azelieic acid, etc., may be thickened by the ureido compounds of the present invention to produce excellent greases. Polyfluoro derivatives of organic compounds, particularly hydrocarbons and dibasic acid esters of H(CF<sub>2</sub>)<sub>n</sub>CH<sub>2</sub>OH, in the lubricating oil viscosity range can be thickened with com-

5 pounds of the present invention. Other synthetic oils, such as esters of aliphatic carboxylic acids and polyhydric alcohol, e.g. trimethylolpropane pelargonate, pentaerythritol hexanoate, can be used as suitable oil vehicles.

#### PREFERRED EMBODIMENT

The following examples are illustrative of a preferred embodiment of the present invention.

#### EXAMPLE I

An ureido compound thickened grease employing "Amine 750" and bitolyene diisocyanate was prepared as follows:

- a. To a grease kettle were added 1,400 gallons of a SAE 10 solvent-extracted base petroleum oil and 262 pounds of bitolyene diisocyanate, the mixture heated to 150° F., and after shutting off the heat the mixture stirred for about one-half hour to dissolve the isocyanate.
- b. The oil solution of the isocyanate is then heated to 210° F. and 660 pounds of "Amine 750" rapidly added to the heated oil solution, and the mixture heated to 385° F. with medium stirring. At 385° F., the heat source is removed, and when the temperature of the batch reaches 390° F. the heated mixture is transferred to a mixer while stirring at low speed. After transfer to the mixer, the transfer line is flushed with 20 gallons of solvent-treated SAE 10 base oil.
- c. The solution in the mixer was cooled to 225° F. and the following additives, 36 pounds of an aromatic amine antioxidant (marketed as "Ortholeum 300"), 180 pounds of zinc naphthenate, 180 pounds of tricresyl phosphate, and 180 pounds of an EP agent (marketed as "Santopoid 23R1" speed for one-half hour, and then milled.
- d. The grease was adjusted to the desired consistency by grading in solvent-extracted SAE 10 base oil.

The thickener concentration was 6.0 percent.

#### EXAMPLE IA

The grease of Example IA was prepared as the grease of Example I except that 0.4 percent (based on the finished grease) of added bitolyene diisocyanate was incorporated along with the additives in step (c). The thickener concentration in this grease was 5.2 percent.

#### EXAMPLE IB

50 The grease of this Example was prepared as the grease of Example IA, except that 0.47 percent bitolyene diisocyanate was incorporated. The thickener concentration of the sample was 5.2 percent.

#### EXAMPLE II

The grease of this Example was prepared as the grease of Example I except that the grease contained no tricresyl phosphate.

#### EXAMPLE IIA

The grease of this Example was prepared as the grease of Example II, except that 0.1 percent added bitolyene diisocyanate was incorporated along with the additives in step (c).

#### EXAMPLE IIB

The grease of this Example was prepared as the grease of Example IIA, but contained 0.2 percent added bitolyene diisocyanate.

#### EXAMPLE IIC

The grease of this Example was prepared as the grease of Example IIA, but contained 0.4 percent added bitolyene diisocyanate.

## EXAMPLE III

The grease of this Example was prepared as the grease of Example II.

## EXAMPLE IIIA

The grease of this Example was prepared as the grease of Example III, but contained 0.4 percent added bitolylen diisocyanate.

The effectiveness of the present invention in improving the yield and properties of ureido compound thickened grease is demonstrated by the data in Table I.

TABLE I

| Sample No. | Percent added bitolylen diisocyanate | Worked penetration <sup>1</sup> | 212° F. oven leakage test percent <sup>2</sup> | ASTM drop point, ° F. | ASTM drop point, ° F. after 400° F. heat treatment |
|------------|--------------------------------------|---------------------------------|------------------------------------------------|-----------------------|----------------------------------------------------|
| I          | 0                                    | 434                             |                                                |                       |                                                    |
| IA         | 0.4                                  | 380                             |                                                |                       |                                                    |
| IB         | 0.47                                 | 372                             |                                                |                       |                                                    |
| II         | 0                                    | 336                             | 3.9                                            | 396                   |                                                    |
| IIA        | 0.1                                  | 320                             | 3.6                                            |                       |                                                    |
| IIB        | 0.2                                  | 322                             | 2.0                                            |                       |                                                    |
| IIC        | 0.4                                  | 312                             | 1.7                                            | 473                   |                                                    |
| III        | 0                                    | 328                             |                                                | 454                   | 416                                                |
| IIIA       | 0.4                                  | 284                             |                                                | 462                   | 480                                                |

<sup>1</sup> ASTM penetration after being worked 60 strokes.

<sup>2</sup> Sixty mesh screen in the shape of a cone is loaded with 10 grams of the grease, and the cone supported in beaker is placed in a 212° F. oven for 24 hours. Oil leakage from the grease collected in the beaker is weighed and the percent oil loss from the grease calculated.

The addition of excess polyisocyanate to ureido compound thickened greases increases the yield, i.e., penetration for a grease thickened content, as demonstrated by penetration data of Table I. Similarly, the above data demonstrate the marked lowering of oil leakage from the grease, as well as improving the drop point of such greases. The data in respect of

Examples III and IIIA demonstrate that the addition of excess polyisocyanate, e.g., bitolylen diisocyanate, imparts a more stable drop point to ureido compound thickened greases.

The percentages given herein and in the appended claims 5 are weight percentages, unless otherwise stated.

Although the present invention has been described in the reference to specific embodiments thereof, the invention is not limited thereto, but includes within its scope such modifications and variations as come within the scope of the appended claims.

We claim:

1. An improvement in a lubricating grease comprising a normally liquid lubricant vehicle thickened with from about 2 percent to about 25 percent, by weight, of at least one ureido 10 compound having the general formula



20 wherein R and R'' are abietyl radicals selected from the group consisting of a dehydroabietyl radical, a dihydroabietyl radical, a tetrahydroabietyl radical and mixtures thereof, and R' is an organic radical selected from the group consisting of an alkylene radical of from one to about 30 carbon atoms and an arylene radical, wherein the improvement comprises the incorporation in said grease of an added amount of from about 0.05 percent to about 2.0 percent of the weight of said grease of a polyisocyanate selected from the group consisting of an aliphatic polyisocyanate and an aromatic polyisocyanate.

25 30 2. The composition of claim 1 wherein said vehicle is a hydrocarbon lubricating oil.

3. The composition of claim 1 wherein said vehicle is an acyclic ester of an aliphatic dicarboxylic acid.

4. The composition of claim 1 wherein said vehicle is a silicone polymer oil in the lubricating oil viscosity range.

35 5. The composition of claim 1 wherein R is a bitolylen radical, and said polyisocyanate is bitolylen diisocyanate.

\* \* \* \* \*

40

45

50

55

60

65

70

75